

## UNITED STATES PATENT OFFICE

2,383,916

## LUBRICANTS

John D. Morgan, South Orange, N. J., assignor to  
Cities Service Oil Company, New York, N. Y., a  
corporation of Pennsylvania

No Drawing. Application July 9, 1942,  
Serial No. 450,287

8 Claims. (Cl. 252—42)

This invention relates to lubricants which are more particularly adapted for low temperature lubrication.

Many machines, such as the aeroplane, truck and automobile, operate in atmospheres which may range in temperature from —50° F. to 200° F. A lubricant which is effective for lubrication in this temperature range should have a comparatively uniform viscosity throughout this temperature range.

The primary object of the present invention is to provide a lubricant and method of lubrication which are effective in a temperature range of —50° F. to 200° F.

Another object of the invention is to provide a lubricant which is stable and non-corrosive and which is capable of withstanding high bearing pressures.

With these and other objects in view the invention consists in the lubricant and method of lubricating hereinafter described and particularly defined in the claims.

I have discovered that the alkyl lactates have physical characteristics which adapt them for lubrication in a range of from —50° F. to 200° F. The lactates which are more particularly adapted as lubricants are the alkyl lactates which are esters of  $\alpha$ -hydroxypropionic acid or lactic acid.

The alkyl lactates, particularly adapted for lubricants, have the following physical properties:

|                       | Boiling point | Flash point | Melting point |
|-----------------------|---------------|-------------|---------------|
| Ethyl lactate.....    | °F. 311       | °F. 129     | °F.           |
| Butyl lactate.....    | 370           | 160         | —45           |
| Isobutyl lactate..... | 350-390       | .....       | .....         |

These alkyl lactates are oily liquids and have the following viscosities:

|                       | Temper-ature | Viscosities in centistokes |
|-----------------------|--------------|----------------------------|
| Ethyl lactate.....    | °F. —40      | 69.5                       |
|                       | 0            | 12.9                       |
|                       | 100          | 1.72                       |
|                       | 200          | .75                        |
| Butyl lactate.....    | —40          | 135                        |
|                       | 0            | 22.3                       |
|                       | 100          | 2.44                       |
|                       | 200          | .93                        |
| Isobutyl lactate..... | —40          | 231                        |
|                       | 0            | 29.1                       |
|                       | 100          | 2.49                       |
|                       | 200          | .93                        |

From an observation of these viscosities it will be seen that all of these lactates have apparently uniform viscosity throughout the range of —40° F. to 200° F.

5 All of the alkyl lactates above mentioned have good lubricating values, that is they have better lubricating values than the regular petroleum lubricating spindle oil having a viscosity of 200 at 100° F. If 3.2%, for example, of ethyl lactate is added to the spindle oil, the load-carrying capacity of the oil will be increased 20%.

By adding one of the well known extreme pressure addition agents to any of these alkyl lactates the load-carrying capacity of the lactate will be raised to a point where it will carry very high bearing pressures. For example with an extreme pressure 4-ball testing machine ethyl lactate would seize at 450 lbs. pressure. By the addition of 1% of Polane, the ester would not seize at 1000 lbs. pressure. It has been found that if 1% of Polane or tricresyl phosphite, or Santolube #261 is added to any of the alkyl lactates the load-carrying capacity would be raised to the point where they would not seize in the 4-ball testing machine at a pressure of 1000 lbs.

20 The ethyl and butyl lactates are well adapted for the manufacture of greases. These lactates with approximately 6% of sodium soap will form a grease that is stable and will not bleed. Preferably the lactate contains 1% of the extreme pressure additive to make the grease an extreme pressure carrying grease. The soap preferably is sodium stearate, although it has been found that sodium oleate or sodium palmitate, or any of the sodium soaps of the fatty acids are adapted for making greases with the ethyl and butyl lactates. Such a grease may consist of approximately 93% of one of these lactates, approximately 6% of sodium stearate, and approximately 1% of an extreme pressure agent.

25 These lactates are neutral and non-corrosive in the metal bearings in which they have been employed and will effectively adhere to the bearings through the temperature range of —40° F. to 200° F.

30 Most of the commonly used extreme pressure addition agents are soluble in the lactates and impart load-carrying capacities to the lactates. Polane is a product sold by the Patent Chemicals Company and is understood to be an ester of a fatty acid or a chlorinated ester of a fatty acid, such as ethyl laurate or chlormethyl stearate. Santolube #261 is manufactured by Monsanto Chemical Company and defined as a metallic

derivative of an alkylated carboxylic acid containing compounds of tin and sulfur. The tricresyl phosphite referred to above is described in the patent to Engelke No. 2,260,303 granted October 28, 1941, and is described as a tricresyl phosphite, or a mixture of tricresyl phosphite and tricresyl phosphate. The above addition agents also act as oiliness and anticorrosion agents.

Certain subject-matter disclosed herein is claimed in divisional application Serial No. 519,649, filed January 25, 1944.

The preferred form of the invention having been thus described, what is claimed as new is:

1. A lubricant consisting essentially of ethyl lactate having approximately 1% of an extreme pressure addition agent dissolved therein.
2. A lubricant comprising ethyl lactate 93%, sodium stearate 6%, tricresyl phosphite 1%.
3. A lubricant comprising ethyl lactate 93 percent, sodium stearate 6 percent, and an extreme pressure addition agent 1 percent.

4. A lubricant consisting essentially of a liquid alkyl lactate having an extreme pressure agent dissolved therein in sufficient proportion to impart extreme pressure properties to the lubricant.

5. A lubricant consisting essentially of a liquid alkyl lactate containing approximately 1% of an extreme pressure agent.

10 6. A lubricant consisting essentially of ethyl lactate having an extreme pressure agent dissolved therein in sufficient proportion to impart extreme pressure properties to the lubricant.

15 7. A lubricant consisting essentially of a liquid alkyl lactate having approximately 6% of sodium soap embodied therein to impart grease characteristics to the lubricant.

8. A lubricant consisting of approximately 6% of sodium stearate, the remainder of the lubricant consisting essentially of ethyl lactate.

20

JOHN D. MORGAN.